# EUROPEAN PATENT SPECIFICATION

(11) **EP 2 101 037 B1**
(45) Date of publication and mention of the grant of the patent: **05.12.2012**
(21) Application number: 09007820.5
(22) Date of filing: 14.07.2006
(51) Int. Cl.: E21B 10/08, E21B 10/20, E21B 10/22

(54) **A method for reducing residual stress in a roller cone bit**
Verfahren zum Reduzieren von Restspannung in einem Rollenmeissel
Procédé permettant de réduire les contraintes résiduelles dans un trépan à molettes coniques

(30) Priority: 15.07.2005 US 183121
(43) Date of publication of application: 16.09.2009
(62) Divisional of application: 06787231.7
(73) Proprietor: Baker Hughes Incorporated, Houston, TX 77019 (US)
(72) Inventor: Zahradnik, Anton F., Sugar Land Texas 77479 (US); Jones, Ronnie L., New Waverly Texas 77358 (US); Nguyen, Don Q., Houston Texas 77066 (US); Ricks, Gregory L., Spring Texas 77386 (US); Beuershausen, Christopher G., Magnolia Texas 77354 (US); Sullivan, Eric C., Houston Texas 77089 (US)
(74) Representative: Jeffrey, Philip Michael

(56) References cited:
- WO-A-99/39075
- JP-A- 11 209 825
- US-A- 3 158 214
- US-A- 3 989 315
- US-A1- 2004 250 584

## Description

The present invention relates in general to stress reduction in roller cone bits and, in particular, to an improved method, and apparatus for reducing residual stress in as-welded roller cone bit ball plug welds.

Rotary-type drill bits include both rotary drag bits and roller-cone bits. In a roller-cone arrangement, the bit typically has three cones, each independently rotatable with respect to the bit body supporting the cones through bearing assemblies. The cones carry either integrally formed teeth or separately formed inserts that provide the cutting action of the bit.

Roller cone bits typically use a ball retention system for securing the cones to the heads. The retention system includes a radial ball race incorporated into each cone and the head bearings. A ball way is provided between the head ball race and the head outer diameter (OD) to facilitate assembly. When the cone is mated to the head, the respective ball races are aligned and, together, they define a toroidal space. Ball bearings are introduced via the ball way into the space. A ball plug is then inserted into the ball way to block the discontinuity (i.e., the hole) in the head ball race and to ensure that the ball bearings are retained in the race. The ball plug is secured to the head OD by welding.

While cooling from welding, residual stress can accumulate in the weld region (e.g., the fusion and heat-affected zones). Depending upon the orientation and magnitude of the residual stress, the service load capacity of the assembly can be significantly reduced. This structural configuration gives rise to one type of head section failure, which includes cracks that initiate at the root of the ball plug weld and then propagate toward the head OD, and then turn and propagate toward the base of the bearing pin. Solutions for addressing this problem would be desirable.

### CLOSEST PRIOR ART DOCUMENT

US 3,989,315 discloses a roller-cone bit wherein the ball plug is secured to the head outer diameter with a mechanically wedged plug.

WO 99/39075 discloses a roller-cone bit wherein the ball plug weld is formed at least in part by a layer of hard facing material.

According to an aspect of the present invention there is provided a method of reducing residual stress in a roller cone bit as claimed in claim 1. According to another aspect of the present invention there is provided a roller cone bit as claimed in claim 11.

One embodiment of a method, and apparatus of the present invention describes a solution for reducing residual stress in the region of as-welded ball plug welds. By reducing weld area residual stress with the present invention, service load capacity and/or service life is increased.

Various embodiments of the present invention will now be described, by way of example only, and with reference to the accompanying drawings in which:
Figure 1 is a half-sectional view of one embodiment of a roller cone bit constructed in accordance with an embodiment of the present invention;
Figure 2 is an enlarged sectional view of a head and cone portion of the roller cone bit of Figure 1 and is constructed in accordance with an embodiment of the present invention;
Figure 3 is an enlarged sectional view of a roller cone bit according to an arrangement; and
Figure 4 is a high level flow diagram of one embodiment of a method constructed in accordance with the present invention.

Referring to Figures 1 and 2, one embodiment of a roller cone bit 11 constructed in accordance with the preferred embodiment of the present invention is shown. Bit 11 comprises a bit body 13 having heads 15 (one shown) with cones 17. Each head 15 and cone 17 includes a retention system having a ball race 19 at an intersection between the head 15 and cone 17. A ball way 21 extends from the ball race 19 to an outer diameter (left sides of Figures 1 and 2) of the head 15. The outer diameter forms a portion of a perimeter area 23 of the head 15. The perimeter area 23 generally includes a region of the head 15 extending from the ball way 21 radially outward and axially inward with respect to the ball way 21.

The respective ball races 19a, 19b of the head 15 and cone 17 are aligned to define a toroidal space. Balls 25 are located in the ball race 19 for mechanically retaining the cone 17 on the head 15. A ball plug 27 is located in the ball way 21 to retain the balls 25 in the ball race 19. A barrier 29, such as a weld, is formed adjacent the outer diameter of the head 15 to secure the ball plug 27 in the ball way 21.

The present invention also comprises stress reduction means for reducing residual stress at the barrier (e.g., weld) 29 and the perimeter area 23 of the head 15 adjacent the outer diameter to increase a service load capacity and a service life of the roller cone bit 11. In one arrangement, the stress reduction means comprises an inner weld 31 (Figure 2) formed from a first material adjacent the ball plug 27. The weld29 is formed on the inner weld 31 from a second material that has a higher strength than the first material. The first material may comprise many different materials, including nickel, nickel alloy, stainless steel, and inconel. The second material may comprise steel or the like.

A single weld comprising one or more passes may be used as the barrier 29. A single material, such as nickel, is utilized to form the welds. Moreover, the entire weld may be formed from a single, softer material. In another arrangement, the stress reduction means comprises a void 39 (Figure 3) in the barrier 29. The void 39 may comprise a drilled hole that extends in an axial direction of the ball way 21.

Also provided herein is a system for reducing residual stress in a roller cone bit 11. One embodiment of the system comprises the elements described above, including the retention system for securing the cones 17 to the heads 15. A residual stress reduction is located at the barrier 29 and the perimeter area 23 to increase a service load capacity and a service life of the roller cone bit 11. The residual stress reduction may comprise an inner weld 31 formed adjacent the ball plug 27 from a first material, and the barrier 29 may comprise an outer weld formed on the inner weld 31 from a second material that has a higher strength than the first material.

The residual stress reduction also may comprise a heat treatment that may be performed on the entire roller cone bit 11. As shown in Figure 3, the residual stress reduction may be localized and limited to the barrier 29 and the perimeter area 23, as with a small device 35 (e.g., a heat source, an ultrasonic tool, etc.) and a controller 37 for applying a heat treatment or an ultrasonic vibration treatment, respectively, to the barrier 29 and the perimeter area 23. Also described above, the residual stress reduction may be accomplished by removing material from the barrier 29, such as by forming a hole 39 in the barrier 29 that extends in an axial direction with respect to the ball way 21.

The present invention also comprises a method of reducing residual stress in a roller cone bit. As shown in Figure 4, one embodiment of the method starts as indicated at step 41, and comprises providing a roller cone bit with heads with cones (step 43); securing the cones to the heads with balls located in a ball race at an intersection between each cone and head, each ball race having a ball way extending from the ball race to a perimeter area of the head (step 45); installing a ball plug in each ball way to retain the balls in the ball race (step 47); forming a barrier at the perimeter area to retain the ball plug in the ball way (step 49); reducing residual stress at the barrier and the perimeter area to increase a service load capacity and a service life of the roller cone bit (step 51); before ending as indicated at step 53.

The method also may comprise forming an inner weld from a first material adjacent the ball plug, and forming an outer weld on the inner weld from a second material that has a higher strength than the first material. Step 51 may comprise applying a heat treatment, such as by subjecting the ball plug to elevated temperatures during the stress relief operation. This embodiment may further comprise localizing the heat treatment to a limited portion of the roller cone bit including the barrier and the perimeter area, or subjecting the entire roller cone bit to the heat treatment. Step 51 also may comprise applying an ultrasonic vibration treatment the barrier and the perimeter area, or removing material from the barrier, such as by forming a hole in the barrier that extends in an axial direction of the ball way.

While the invention has been shown or described in only some of its forms, it should be apparent to those skilled in the art that it is not so limited, but is susceptible to various changes without departing from the scope of the invention.

## Claims

1. A method of reducing residual stress in a roller cone bit, the method comprising:
(a) providing a roller cone bit (11) with heads (15) with cones (17);
(b) securing the cones (17) to the heads (15) with balls (25) located in a ball race (19) at an intersection between each cone and head, each ball race (19) having a ball way (21) extending from the ball race to a perimeter area (23) of the head (15);
(c) installing a ball plug (27) in each ball way (21) to retain the balls (25) in the ball race (19); and
(d) forming a barrier (29) at the perimeter area (23) to retain the ball plug (27) in the ball way (21) by forming a weld;
**characterised in that** the weld is formed from a single material selected from the group consisting of: (i) stainless steel; and (ii) Inconel.

2. A method according to claim 1, wherein said weld (29) is formed from Inconel.

3. A method according to claim 1 or 2, wherein said weld (29) comprises a single weld.

4. A method according to claim 3, comprising forming the single weld (29) with at least one pass from the single material.

5. A method according to any preceding claim, further comprising applying a stress relief operation with heat treatment to reduce residual stress in the barrier (29) and the perimeter area (23) of the roller cone bit (11).

6. A method according to claim 5, comprising subjecting the ball plug (27) to elevated temperatures during the stress relief operation.

7. A method according to claim 5, comprising localizing the heat treatment to a limited portion of the roller cone bit (11) including the barrier (29) and the perimeter area (23).

8. A method according to claim 5, comprising subjecting the entire roller cone bit (11) to the heat treatment.

9. A method according to any of claims 1 to 4, further comprising applying an ultrasonic vibration treatment to the barrier (29) and the perimeter area (23) to reduce residual stress in the barrier (29) and the perimeter area (23) of the roller cone bit (11).

10. A method according to any preceding claim, wherein residual stress in the barrier (29) and the perimeter area (23) is reduced to increase a service load capacity and a service life of the roller cone bit (11).

11. A roller cone bit, comprising:
a bit body (13) having heads (15) with cones (17), each head and cone including a ball race (19) at an intersection between the head (15) and cone (17);
a ball way (21) extending from the ball race (19) to an outer diameter of the head (15), the respective ball races of the head and cone being aligned to define a toroidal space;
balls (25) located in the ball race (19) for mechanically retaining the cone (15) on the head (17);
a ball plug (27) located in the ball way (21) to retain the balls (25) in the ball race (19); and
a weld (29) formed adjacent the outer diameter of the head (15) to secure the ball plug (27) in the ball way (21);
**characterised in that** the weld (29) is formed from a single material selected from the group consisting of: (i) stainless steel; and (ii) Inconel.

12. A roller cone bit according to claim 11, wherein said weld (29) is formed from Inconel.

13. A roller cone bit according to claim 11 or 12, wherein said weld (29) comprises a single weld.

## Patentansprüche

1. Verfahren zum Verringern der Restbeanspruchung in einem Rollenmeißel, wobei das Verfahren Folgendes umfasst:
(a) Vorsehen eines Rollenmeißels (11) mit Köpfen (15) mit Konussen (17);
(b) Befestigen der Konusse (17) an den Köpfen (15) mit Kugeln (25), die sich in einer Kugellaufbahn (19) an einer Schnittfläche zwischen jedem Konus und
dem Kopf befinden, wobei jede Kugellaufbahn (19) eine Kugelbahn (21) besitzt, die von der Kugellaufbahn zu einem Umfangsbereich (23) des Kopfes (15) verläuft;
(c) Installieren eines Kugelstopfens (27) in jeder Kugelbahn (21), um die Kugeln (25) in der Kugellaufbahn (19) zu halten; und
(d) Bilden einer Sperre (29) in dem Umfangsbereich (23), um den Kugelstopfen (27) in der Kugelbahn (21) zu halten, indem eine Schweißnaht gebildet wird;
**dadurch gekennzeichnet, dass** die Schweißnaht aus einem einzigen Material gebildet wird, das aus der Gruppe gewählt wird, die besteht aus: (i) Edelstahl; und (ii) Inconel.

2. Verfahren nach Anspruch 1, wobei die Schweißnaht (29) aus Inconel gebildet wird.

3. Verfahren nach Anspruch 1 oder 2, wobei die Schweißnaht (29) eine einzige Schweißnaht umfasst.

4. Verfahren nach Anspruch 3, wobei das Bilden der einzigen Schweißnaht (29) in wenigstens einem Durchgang aus dem einzigen Material gebildet wird.

5. Verfahren nach einem vorhergehenden Anspruch, das ferner das Anwenden einer Beanspruchungsentlastungsoperation mit Wärmebehandlung umfasst, um die Restbeanspruchung in der Sperre (29) und dem Umfangsbereich (23) des Rollenmeißels (11) zu verringern.

6. Verfahren nach Anspruch 5, das das Beaufschlagen des Kugelstopfens (27) mit erhöhten Temperaturen während der Beanspruchungsentlastungsoperation umfasst.

7. Verfahren nach Anspruch 5, das das räumliche Einschränken der Wärmebehandlung auf einen begrenzten Abschnitt des Rollenmeißels (11), der die Sperre (29) und den Umfangsbereich (23) enthält, umfasst.

8. Verfahren nach Anspruch 5, das das Beaufschlagen des gesamten Rollenmeißels (11) mit der Wärmebehandlung umfasst.

9. Verfahren nach einem der Ansprüche 1 bis 4, das ferner das Anwenden einer Ultraschallvibrationsbehandlung auf die Sperre (29) und den Umfangsbereich (23) umfasst, um die Restbeanspruchung in der Sperre (29) und dem Umfangsbereich (23) des Rollenmeißels (11) zu verringern.

10. Verfahren nach einem vorhergehenden Anspruch, wobei die Restbeanspruchung in der Sperre (29) und dem Umfangsbereich (23) verringert wird, um eine Arbeitslastkapazität und eine Arbeitslebensdauer des Rollenmeißels (11) zu erhöhen.

11. Rollenmeißel, der Folgendes umfasst:
einen Meißelkörper (13), der Köpfe (15) mit Konussen (17) besitzt, wobei jeder Kopf und jeder Konus an einer Schnittfläche zwischen dem Kopf (15) und dem Konus (17) eine Kugellaufbahn (19) enthalten;
eine Kugelbahn (21), die von der Kugellaufbahn (19) zu einem äußeren Durchmesser des Kopfes (15) verläuft, wobei die jeweiligen Kugellaufbahnen des Kopfes und des Konus aufeinander ausgerichtet sind, um einen toroidförmigen Raum zu definieren;
Kugeln (25), die sich in der Kugellaufbahn (19) befinden, um den Konus (15) an dem Kopf (17) mechanisch zu halten;
einen Kugelstopfen (27), der sich in der Kugelbahn (21) befindet, um die Kugeln (25) in der Kugellaufbahn (19) zu halten; und
eine Schweißnaht (29), die in der Nähe des äußeren Durchmessers des Kopfes (15) gebildet ist, um den Kugelstopfen (27) in der Kugelbahn (21) zu befestigen;
**dadurch gekennzeichnet, dass** die Schweißnaht (29) aus einem einzigen Material gebildet ist, das aus der Gruppe gewählt ist, die besteht aus: (i) Edelstahl; und (ii) Inconel.

12. Rollenmeißel nach Anspruch 11, wobei die Schweißnaht (29) aus Inconel gebildet ist.

13. Rollenmeißel nach Anspruch 11 oder 12, wobei die Schweißnaht (29) eine einzige Schweißnaht umfasst.

## Revendications

1. Procédé permettant de réduire les contraintes résiduelles dans un trépan à molettes coniques, le procédé comprenant les étapes consistant à :
(a) fournir un trépan à molettes coniques (11) pourvu de têtes (15) comportant des cônes (17) ;
(b) assujettir les cônes (17) aux têtes (15) au moyen de billes (25) situées dans une piste de roulement (19) à billes à une intersection entre chaque cône et chaque tête, chaque piste de roulement (19) à billes comprenant un chemin de roulement (21) à billes qui s'étend depuis la piste de roulement à billes jusqu'à une région périphérique (23) de la tête (15) ;
(c) installer un obturateur (27) de billes dans chaque chemin de roulement (21) à billes pour retenir les billes (25) dans la piste de roulement (19) à billes ; et
(d) former une barrière (29) au niveau de la région périphérique (23) pour retenir l'obturateur (27) de billes dans le chemin de roulement (21) à billes en formant une soudure ;
**caractérisé en ce que** la soudure est formée à partir d'un matériau unique sélectionné parmi le groupe constitué de : (i) acier inoxydable; et (ii) Inconel.

2. Procédé selon la revendication 1, dans lequel ladite soudure (29) est formée d'Inconel.

3. Procédé selon la revendication 1 ou 2, dans lequel ladite soudure (29) comprend une soudure unique.

4. Procédé selon la revendication 3, comprenant la formation de la soudure unique (29) en au moins une passe à partir du matériau unique.

5. Procédé selon l'une quelconque des revendications précédentes, comprenant en outre l'application d'une opération de détente à traitement thermique pour réduire les contraintes résiduelles dans la barrière (29) et la région périphérique (23) du trépan à molettes coniques (11).

6. Procédé selon la revendication 5, comprenant l'étape consistant à soumettre l'obturateur (27) de billes à des températures élevées pendant l'opération de détente.

7. Procédé selon la revendication 5, comprenant l'étape consistant à circonscrire le traitement thermique à une partie limitée du trépan à molettes coniques (11) qui comprend la barrière (29) et la région périphérique (23).

8. Procédé selon la revendication 5, comprenant l'étape consistant à soumettre la totalité du trépan à molettes coniques (11) au traitement thermique.

9. Procédé selon l'une quelconque des revendications 1 à 4, comprenant en outre l'étape consistant à appliquer un traitement de vibration ultrasonique à la barrière (29) et à la région périphérique (23) pour réduire les contraintes résiduelles dans la barrière (29) et la région périphérique (23) du trépan à molettes coniques (11).

10. Procédé selon l'une quelconque des revendications précédentes, les contraintes résiduelles dans la barrière (29) et la région périphérique (23) étant réduites dans le but d'accroître une capacité de charge d'exploitation et une durée de vie utile du trépan à molettes coniques (11).

11. Trépan à molettes coniques, comprenant :
un corps (13) de trépan pourvu de têtes (15) comportant des cônes (17), chaque tête et chaque cône comprenant une piste de roulement (19) à billes à une intersection entre la tête (15) et le cône (17) ;
un chemin de roulement (21) à billes qui s'étend depuis la piste de roulement (19) à billes jusqu'à un diamètre extérieur de la tête (15), les pistes de roulement à billes respectives de la tête et du cône étant alignées pour délimiter un espace toroïdal ;
des billes (25) situées dans la piste de roulement (19) à billes pour retenir mécaniquement le cône (15) sur la tête (17) ;
un obturateur (27) de billes situé dans le chemin de roulement (21) à billes pour retenir les billes (25) dans la piste de roulement (19) à billes ; et une soudure (29) formée en position adjacente au diamètre extérieur de la tête (15) pour assujettir l'obturateur (27) de billes dans le chemin de roulement (21) à billes ;
**caractérisé en ce que** la soudure (29) est formée à partir d'un matériau unique choisi parmi le groupe constitué de : (i) acier inoxydable; et (ii) Inconel.

12. Trépan à molettes coniques selon la revendication 11, dans lequel ladite soudure (29) est formée d'Inconel.

13. Trépan à molettes coniques selon la revendication 11 ou 12, dans lequel ladite soudure (29) comprend une soudure unique.
